

Patented Mar. 6, 1928.

1,661,515

# UNITED STATES PATENT OFFICE.

OTTO TREICHEL, OF BERLIN, GERMANY.

## PROCESS OF PRINTING IN GREASY INKS WITH GELATIN PRINTING SURFACES.

No Drawing. Application filed November 30, 1926, Serial No. 151,826, and in Germany December 18, 1925.

It is well known that in the process of printing in greasy inks with gelatin printing surfaces, more or less elevated reliefs are formed under the action of the wetting medium, said reliefs being undesirable in that they cause trouble during the distribution of the ink as well as during the actual printing. Several attempts have already been made to remove this drawback but none of them have had the desired result.

The present invention strikes out in a new direction, in that the evil is attacked at the root and the gelatin is treated at the outset in such a manner that its swelling capacity is reduced.

The process consists in this that to the gelatin are added by way of the wetting medium, substances which reduce the swelling property of the gelatin, for instance, 20 solutions of sodium sulphate. A decinormal solution of the wetting medium is mentioned as a proportion which has proved satisfactory in practice.

It is obvious that by means of this treatment also the subsequently formed relief, which can never be entirely avoided, is very considerably reduced. It is true that in the reliefs so produced, the high lights also take up greasy inks; this is obviated according to the invention by increasing the temperature of the wetting medium. Normally a wetting medium at 22° is employed. According to the invention, temperatures of about 25° and over are employed. A further advantage of the new process consists in this that in the well-known interdependence of the relief with the gradation, the latter can be adjusted to any desired degree.

In the appended claims, by the term "a

substance having the property of reducing 40 or delaying the swelling of the gelatin" I mean to include all salts such as sulphates, citrates, acetates, salts of di- and multi-valent cations, etc. all of which possess the well known and common property of reducing 45 or delaying gelatin swelling.

Having now particularly described and ascertained the nature of my said invention and in what manner the same is to be performed, I declare that what I claim is:— 50

1. In the process of printing with greasy inks on gelatin printing surfaces, the step consisting in wetting the gelatin printing surface with a wetting medium containing 55 a substance having the property of reducing or delaying the swelling of the gelatin.

2. In the process of printing with greasy inks on gelatin printing surfaces, the step consisting in treating the gelatin with a substance having the property of reducing or 60 delaying the swelling of the gelatin.

3. In the process of printing with greasy inks on gelatin printing surfaces, the step consisting in wetting the gelatin printing 65 surface with a wetting medium containing sodium sulphate, for the purpose set forth.

4. In the process of printing with greasy inks on gelatin printing surfaces, the step consisting in wetting the gelatin printing surface with a wetting medium heated to a 70 temperature above 22° C., and containing a substance having the property of reducing or delaying the swelling of the gelatin for the purpose set forth.

In testimony whereof I have signed my 75 name to this specification.

DR. O. TREICHEL.